

## UNITED STATES PATENT OFFICE

2,656,271

METHOD OF DEVELOPING AGED PHOTO-  
SENSITIVE MATERIAL CONTAINING SIL-  
VER HALIDE AND A CHROMATEWilhelm Neugebauer and Maximilian Karl  
Reichel, Wiesbaden-Biebrich, Germany, assign-  
ors to Keuffel & Esser Company, Hoboken, N. J.No Drawing. Application October 13, 1950, Se-  
rial No. 190,041. In Germany October 24, 1949.

8 Claims. (Cl. 95—88)

## 1

This invention relates to photosensitive layers of a type which are commercially applied to tracing cloth or the like to produce photosensitive materials used as intermediates in the reproduction of drawings. This type of photosensitive material serves as a duplicate tracing from which prints can be made in the usual manner. More particularly the invention relates to photosensitive layers made up of a colloid (such as glue or the like), an agent capable of hardening the colloid upon exposure to light (such as chromate salts), and a silver halide.

When this type of material is exposed to light, the colloid later is hardened in the exposed areas and a latent silver halide image is also formed. The material is developed by rubbing with water to remove the colloid layer from the unexposed areas and it is then developed to convert the silver halide to a black silver image in the exposed areas.

These materials have the disadvantage however that their "shelf life" or "keeping quality" is poor. For this reason it is necessary to use these materials a short time after the photosensitive colloid layer has been coated on the base sheet even if they were stored under conditions of low temperature and humidity. Material which was stored too long under unfavorable conditions had to be discarded because it did not give satisfactory prints.

Now it has been found that satisfactory prints can be obtained on material of this type even after months of storage under conditions which formerly would have made the material unusable, if the exposed material is subjected during the development of the exposed material, to the influence of certain mono-nitro-substituted heterocyclic compounds constituted in such a manner that a benzene or naphthalene nucleus is condensed together with a five-membered closed heterocyclic chain selected from the group consisting of



The position of the nitro group is preferably in the benzene and naphthalene nucleus, respectively.

## 2

The heterocyclic nitro compound is caused to react with the light-exposed material preferably in a weakly alkaline solution.

Compounds which may be used in accordance with this invention are, for example, mono-nitro-benzimidazoles, mono-nitro-benzotriazoles, mono-nitro-benzopyrazoles, mono-nitro-benzothiazoles, mono-nitro-naphthoimidazoles, and mono-nitro-naphthotriazoles. If for example 0.1% of 6-nitro-benzimidazole is added to a soda-alkaline metal hydroquinone developing solution, the unexposed areas of the material developed therewith are free of silver-fog, even if the photosensitive layer on the material is so decomposed that it would normally have given an almost entirely black print.

Furthermore, it has been found that the sulfonation products of the mono-nitro-substituted heterocyclic compounds of the naphthalene series which may be used in accordance with this invention for the treatment of light-exposed colloid layers containing silver halide and a chromate, yield equally good results. The sulfonation products are preferably used as alkali metal salts.

It is important that the mono-nitro-substituted heterocyclic compound be applied in the developing solution. Addition of the compound to the photosensitive colloid layer is not effective, apparently because of the chromates present therein.

However, when a developing solution containing a compound of this type is used on decomposed photosensitive material of the kind described a disturbing reddish discoloration of the background occurs. In order to avoid this it is necessary to give the developed material a quick treatment with an acid fixing bath.

Images having high contrast are obtained from photo-sensitive material containing a hardenable colloid such as glue, silver halide and chromate by development according to this invention, even if the material has been stored for months or under forced conditions, for example for 72 hours at 40° C. in air containing 90% relative humidity.

In order to illustrate the present invention the following examples are inserted:

(1.) A light-sensitive photosensitive intermediate material is prepared by coating tracing

cloth waterproofed with a nitrocellulose lacquer with an aqueous colloidal dispersion containing the following ingredients:

- 5 liquid ounces of Le Pages photographic glue (fish glue),  
 9 liquid ounces of silver nitrate solution (3.07 ounces of C. P. salt in distilled water),  
 9 liquid ounces of potassium chloride solution (1.43 ounces of C. P. salt in distilled water),  
 77 liquid ounces of distilled water,  
 9 liquid ounces of ammonium bichromate (11 grams of C. P. salt in distilled water).

The material is stored for 72 hours under forced conditions (40° C. 90% relative humidity) and subsequently exposed to light under a suitable master. Thereafter the material is developed with an aqueous solution containing the following ingredients:

- 4 grams of metol,  
 12 grams of hydroquinone,  
 12 grams of sodium carbonate (water free),  
 44 grams of sodium sulfite (crystallized),  
 2.25 grams of 6-nitro-benzimidazole (total volume=2250 ccm.).

A deep black silver image on a background free of fog is obtained. If the developer solution is used without the addition of 6-nitro-benzimidazole, a deep black silver layer covers the whole surface of the image making it impossible to distinguish any details of the negative image.

In order to avoid the formation of the disturbing reddish discoloration of the background, the above described copies of high contrast are quickly treated with an acid fixing bath having the following composition:

- 50 grams of sodium sulfite (crystallized),  
 15 grams of tartaric acid,  
 200 grams of sodium thiosulfate (crystallized) in 1000 ccm. of distilled water, total volume.

Subsequently the copies are washed and dried.

The waterproofed tracing cloth base material may be replaced by a cellulose acetate foil saponified on its surface or even by metallic foils, for example, an aluminum foil or a zinc foil. Metallic foils, for example aluminum foils which have been covered with a surface layer consisting of metal oxide or metallic foils provided with a solid porous coating consisting of fluorine or phosphorous compounds provide a particularly good base material for the photosensitive layer and excellent prints can be made thereon.

(2.) The same colloidal layer as described in Example 1 containing fish glue, silver salt and dichromate is used for the preparation of the photosensitive layer on a suitable base, but in lieu of 2.25 grams of 6-nitro-benzimidazole 2.25 grams of 6-nitro-benzotriazole are added to the developer solution.

(3.) The same colloidal layer as described in Example 1 containing fish glue, silver salt and dichromate is used for the preparation of the photosensitive layer on a suitable base, but instead of 2.25 grams of 6-nitro-benzimidazole 2.25 grams of 6-nitro-benzopyrazole are added to the developer solution.

(4.) The same colloidal layer as described in Example 1 containing fish glue, silver salt and dichromate is used for the preparation of the photosensitive layer on a suitable base, but instead of 2.25 grams of 6-nitro-benzimidazole 3.75 grams of sodium 6-nitro-1,2-naphthoimidazole sulfonate are added to the developer solution.

(5.) The same colloidal layer as described in

Example 1 containing fish glue, silver salt and dichromate is used for the preparation of the photosensitive layer on a suitable base, but in lieu of 2.25 grams of 6-nitro-benzimidazole a mixture consisting of 1.87 grams of sodium 6-nitro-naphthoimidazole sulfonate and 1.12 grams of 6-nitro-2-hydroxy-benzothiazole are added to the developer solution.

(6.) The same colloidal layer as described in Example 1 containing fish glue, silver salt and dichromate is used for the preparation of the photosensitive layer on a suitable base, but instead of 2.25 grams of 6-nitro-benzimidazole 3.75 grams of sodium 6-nitro-1,2-naphthotriazole sulfonate are added to the developer solution.

After having fully described and explained our present invention, what we claim is:

1. The method of producing images rich in contrast from aged photosensitive material comprising a colloid layer containing silver halide and a chromate on a base, which comprises treating said material after its exposure to light under a master with a developing solution containing a reducing agent for the exposed silver halide and a mono-nitro-substituted heterocyclic compound selected from the group of nitro substituted benzene and nitro substituted naphthalene condensed with a five-membered closed heterocyclic chain selected from the group consisting of



2. The method of producing images rich in contrast, from aged photosensitive material comprising a colloid layer containing silver halide and a chromate on a base, which comprises treating said material after its exposure to light under a master with a developing solution containing a reducing agent for the exposed silver halide and a sulfonation product of a mono-nitro-substituted heterocyclic compound selected from the group of nitro substituted naphthalene condensed with a five-membered closed heterocyclic chain selected from the group consisting of



3. The method of producing images rich in contrast, from aged photosensitive material comprising a colloid layer containing silver halide and a chromate on a base, which comprises treating said material after its exposure to light under a master with a developing solution containing a reducing agent for the exposed silver halide and 6-nitro-benzimidazole.

4. The method of producing images rich in contrast, from aged photosensitive material comprising a colloid layer containing silver halide and a chromate on a base, which comprises treating said material after its exposure to light under a master with a developing solution containing a reducing agent for the exposed silver halide and 6-nitro-benzotriazole.

5. The method of producing images rich in contrast, from aged photosensitive material comprising a colloid layer containing silver halide and a chromate on a base, which comprises treating said material after its exposure to light under a master with a developing solution containing a reducing agent for the exposed silver halide and 6-nitro-benzopyrazole.

6. The method of producing images rich in contrast, from aged photosensitive material comprising a colloid layer containing silver halide and a chromate on a base, which comprises treating said material after its exposure to light under a master with a developing solution containing a reducing agent for the exposed silver halide and 6-nitro-1,2-naphthoimidazole-sulfonic acid alkali salt.

7. The method of producing images rich in contrast, from aged photosensitive material comprising a colloid layer containing silver halide and a chromate on a base, which comprises treating said material after its exposure to light under a master with a developing solution containing a reducing agent for the exposed silver halide and 6-nitro-1,2-naphthotriazole-sulfonic acid alkali salt.

8. The method of producing images rich in contrast from aged photosensitive material comprising a colloid layer containing silver halide and a chromate on a base, which comprises treating said material after its exposure to light under a master with a developing solution containing a reducing agent for the exposed silver

10  
15  
20  
25

halide and a mono-nitro-substituted heterocyclic compound selected from the group of nitro substituted benzene and nitro substituted naphthalene condensed with a five-membered closed heterocyclic chain selected from the group consisting of



and the sulfonation products of said mono-nitro-substituted heterocyclic compounds of the naphthalene series and then treating said material with an acid fixing bath.

WILHELM NEUGEBAUER.  
MAXIMILIAN KARL REICHEL.

References Cited in the file of this patent

UNITED STATES PATENTS

| Number    | Name     | Date           |
|-----------|----------|----------------|
| 2,271,229 | Peterson | Jan. 27, 1942  |
| 2,384,593 | Bean     | Sept. 11, 1945 |
| 2,497,917 | Stauffer | Feb. 21, 1950  |